

April 29, 1947.

C. J. QUIGLEY

2,419,591

MAGNETIC MINESWEEPING ELECTRODE CABLE

Filed Nov. 5, 1943



CHARLES J. QUIGLEY  
INVENTOR  
BY *John T. Quigley*  
ATTORNEY

## UNITED STATES PATENT OFFICE

2,419,591

MAGNETIC MINESWEEPING ELECTRODE  
CABLE

Charles J. Quigley, United States Navy

Application November 5, 1943, Serial No. 509,084

6 Claims. (Cl. 174—128)

(Granted under the act of March 3, 1883, as  
amended April 30, 1928; 370 O. G. 757)

1

This invention relates to a magnetic minesweeping cable electrode, and has for an object to provide an improved magnetic minesweeping cable electrode which will have considerably longer life than the present conventional magnetic minesweeping cable.

Conventional cables for the same purpose are generally wound from copper wires which are applied in layers until the proper dimension of cable is attained. A typical cable is one made of one-eighth inch diameter wire applied in layers of 1, 6, 12 and 18 and 24 wires per layer, respectively, from the center outward. A disadvantage of such minesweeping cable electrode is its short life. Such copper cable electrodes are badly attacked by the products of the electrolysis of salt water occurring during the passage of heavy electrical currents through the sea water between the electrodes. This attack results in the formation of insoluble copper compounds, some of which wash away in the water and represent permanent loss to the electrodes.

It is an object of this invention to avoid such a disadvantage and to lengthen the life of the minesweeping cable electrode very considerably.

A further object of this invention is to provide a magnetic minesweeping cable electrode which not only has far longer life and electrical properties than the conventional cable previously used for this purpose, but also uses considerably less copper in its composition, thus resulting in the saving of this critical material.

This invention is accomplished by omitting the outer layer of copper wires from the cable and substituting instead a peripheral layer of steel wires of the same number and dimension as the eliminated copper wire. The inventor is aware of U. S. Patent to Edwards, No. 2,250,907, of July 29, 1941, but while such patent consists of a cable of both steel and copper strands, such patented cable is not usable for a magnetic minesweeping cable electrode, for its construction is such that its life would be no longer than that of the conventional all copper cable, which the cable of this invention replaces. The particular feature provided by this invention is the provision of a conductive protective coating on the copper wires. The inventor is also aware of the pending patent application to W. L. Williams, Jr., Serial No. 484,855, filed April 28, 1943, now Patent No. 2,396,734, of March 19, 1946, and the present invention is an improvement over such Williams application in that it makes the life of the Williams electrode even greater.

With the foregoing and other objects in view, **55** and reduction during electrolysis. In general, the

2

the invention consists in the construction, combination and arrangement of the parts herein-after described and illustrated in the drawings.

The figure is a cross-sectional view of a magnetic minesweeping cable electrode made up according to this invention.

There is shown at **10** the magnetic minesweeping cable electrode of this invention. This electrode **10** consists of a plurality of layers of individual wires similar in dimension and number to that of the conventional all copper magnetic minesweeping cable electrode, whereas it may be made up of layers of 1, 6, 12, 18 and 24 wires per layer, respectively, from the center outward. All **15** the inner layers **11** of the wire are made of copper just as in the conventional cable, but the outer or peripheral layer **12** is made up of steel wires of the same dimension as the wires **11**, and hence in the cable illustrated there are twenty-four steel wires **12** forming the periphery of its cable. However, if there are a greater or lesser number of layers in the cable, the essential feature is that the peripheral layer or layers should be of steel wires while the inner layers are of copper wire. **20** As a result of this construction it has been found that when the peripheral layer is made of steel or of other ferrous metals or alloys, and the inner layers are made of copper, that there is a considerable increased resistance to metal loss. **25** Typical results of tests made with steel wires **12** wound on copper wires **11** show that with the all copper electrode the weight loss in grams per faraday is 21.3, while under the same conditions the total weight loss in grams per faraday for the **30** steel periphery copper center cable electrode of this invention is only 3.5, the total copper loss being 0.6. The features thus far described are those of the Williams electrode of the above mentioned application. Provision of this invention **35** consists in adding conductive protective coating **14**, particularly about the individual strands of copper wire **11**. This conductive protective coating consists of an inert conductive filler compounded with a plastic binder. This inert filler **40** may be graphite so that the composition of the coating would be graphite and plasticized vinyl chloride in the ratio fifteen to one by weight. Carrying forward the above tests the total weight loss of this invention in grams per faraday is only 2.9, while the total copper loss in grams per faraday **45** is zero. The essential properties of this coating are its excellent electrical conductivity, permanent flexibility under all test conditions, strong adhesion to copper and stability under oxidation **50** and reduction during electrolysis. In general, the

class of plastic binders preferred would be synthetic elastomers similar in properties to plasticized vinyl chloride.

Besides thus possessing a longer life than the all copper cable, its use provides a considerable conservation of copper. The bi-metal electrode of this invention is considerably less expensive and has the necessary properties of high electrical conductivity, high resistance against metal loss, flexibility and ease of handling. Furthermore, the present electrode can be substituted for the all copper electrode and used in the same magnetic minesweeping gear in which the all copper electrode is used without any alterations. The coating may be applied readily and can be 15 repaired on shipboard.

Other modifications and changes in the number and proportions of the parts may be made by those skilled in the art without departing from the nature of this invention within the 20 scope of what is hereinafter claimed.

The invention described herein may be manufactured and used by or for the Government of the United States of America for governmental purposes without the payment of any royalties thereon or therefor.

What is claimed is:

1. A magnetic minesweeping underwater electrode comprising a plurality of layers of wires, the center of the electrode consisting of wires of cuprous materials covered with a conductive corrosion protective coating and the periphery of the electrode consisting of wires of ferrous materials.

2. A magnetic minesweeping underwater electrode made up of a plurality of concentric layers of wires, the inner layers being of copper wire covered with a conductive corrosion protective coating and the periphery of the electrode being of steel wires.

3. A magnetic minesweeping underwater electrode comprising a plurality of layers of wires, the center of the electrode consisting of wires of cuprous materials covered with a conductive corrosion protective coating and the periphery of the electrode consisting of wires of ferrous materials, said conductive protective coating comprising an inert conductive filler combined with a plastic binder.

4. A magnetic minesweeping underwater elec- 50

trode comprising a plurality of layers of wires, the center of the electrode consisting of wires of cuprous materials covered with a conductive corrosion protective coating and the periphery of the electrode consisting of wires of ferrous materials, said conductive corrosion protective coating comprising an inert conductive filler combined with a plastic binder, said inert conductive filler being graphite.

5. A magnetic minesweeping underwater electrode comprising a plurality of layers of wires, the center of the electrode consisting of wires of cuprous materials covered with a conductive corrosion protective coating and the periphery of the electrode consisting of wires of ferrous materials, said conductive corrosion protective coating comprising an inert conductive filler combined with a plastic binder, said plastic binder being plasticized vinyl chloride.

6. A magnetic minesweeping underwater electrode comprising a plurality of layers of wires, the center of the electrode consisting of wires of cuprous materials covered with a conductive corrosion protective coating and the periphery of the electrode consisting of wires of ferrous materials, said conductive corrosion protective coating comprising an inert conductive filler combined with a plastic binder, said inert conductive filler being graphite, said plastic binder being plasticized vinyl chloride, and said graphite and said plasticized vinyl chloride being in the ratio of fifteen to one by weight.

CHARLES J. QUIGLEY.

#### REFERENCES CITED

The following references are of record in the file of this patent:

#### UNITED STATES PATENTS

| Number    | Name        | Date          |
|-----------|-------------|---------------|
| 1,987,508 | Johns       | Jan. 8, 1935  |
| 2,231,595 | Safford     | Feb. 11, 1941 |
| 1,691,869 | Fowle       | Nov. 13, 1928 |
| 2,041,213 | Schellenger | May 19, 1936  |

#### FOREIGN PATENTS

| Number  | Country | Date          |
|---------|---------|---------------|
| 304,031 | British | Jan. 17, 1929 |
| 549,269 | British | 1942          |